

Dec. 30, 1924.

1,521,294

J. C. HENDERSON

# METHOD AND APPARATUS FOR DRAWING SHEET GLASS

Filed Nov. 10, 1923

3 Sheets-Sheet 1



**Inventor**

JOHN C. HENDERSON.

By Attorney *A. P. Rowley*

Dec. 30, 1924.

1,521,294

J. C. HENDERSON

METHOD AND APPARATUS FOR DRAWING SHEET GLASS

Filed Nov. 10, 1923

3 Sheets-Sheet 2



By Attorney C. A. Paisley

Dec. 30, 1924.

1,521,294

J. C. HENDERSON

METHOD AND APPARATUS FOR DRAWING SHEET GLASS

Filed Nov. 10, 1923

3 Sheets-Sheet 3



Inventor  
JOHN C. HENDERSON.

By Attorney C. A. Rowley

Patented Dec. 30, 1924.

1,521,294

## UNITED STATES PATENT OFFICE.

JOHN C. HENDERSON, OF NEW YORK, N. Y., ASSIGNOR TO THE LIBBEY-OWENS SHEET GLASS COMPANY, OF TOLEDO, OHIO, A CORPORATION OF OHIO.

### METHOD AND APPARATUS FOR DRAWING SHEET GLASS.

Application filed November 10, 1923. Serial No. 673,882.

To all whom it may concern:

Be it known that I, JOHN C. HENDERSON, a citizen of the United States, residing at New York, in the county of New York and

5 State of New York, have invented new and useful Improvements in Methods and Apparatus for Drawing Sheet Glass, of which the following is a specification.

This invention relates to the art of drawing 10 a continuous sheet of glass, and more particularly to an improved method and apparatus for bending the plastic glass sheet from one plane to another without injuring the surfaces thereof.

15 In certain well-known systems for producing sheet glass, for example the Colburn process as set forth in the Colburn Patent, 1,248,809, granted December 4, 1917, the glass sheet is drawn upwardly from a pool 20 of molten glass and then, while partially set but still somewhat plastic, is bent through approximately 90° into the horizontal plane where it is carried away through suitable drawing and flattening mechanism into a leer. While being bent from the vertical to the horizontal plane, the sheet is supported 25 upon some form of bending member, usually a highly polished metal roller. It is essential that the cylindrical sheet-supporting 30 surface of this roller be absolutely smooth, clean, and maintained at just the proper temperature, else the delicate fire-polished surface of the plastic sheet will be injured while passing over the roller.

35 In order to avoid the difficulties incident to the use of such a bending member, the present system has been devised. According to the present invention, the plastic sheet, after becoming partially set, is gripped adjacent its edges, and supported by, suitable gripping members which move with the sheet during its bending period. Preferably the sheet edge is gripped between a pair of suitably guided and driven endless chains.

45 These chain loops are so mounted that the sheet-gripping runs of the two opposite chains diverge from one another as they move with the sheet so that a constantly increasing lateral tension is applied to the 50 glass sheet throughout the bending operation. This lateral tension will prevent sagging of the unsupported main central portion of the sheet, which is carried from the

vertical into the horizontal plane without contacting with any solid bodies which 55 might otherwise injure the delicate fire-polished surface of the sheet.

The objects and advantages of this invention will be more clearly understood from the following detailed description of 60 an approved form of the apparatus embodying the principles of this invention.

In the accompanying drawings:

Fig. 1 is a vertical longitudinal section 65 through the apparatus, taken substantially on the line 1—1 of Fig. 2.

Fig. 2 is a plan view of the apparatus, the lower portion of the figure being in section substantially on the line 2—2 of Fig. 1.

Fig. 3 is a transverse vertical section, 70 taken substantially on the line 3—3 of Fig. 1.

Fig. 4 is a transverse vertical section of one side of the apparatus, taken substantially on the line 4—4 of Fig. 1.

Fig. 5 is a view, on an enlarged scale, of 75 a fragment of one pair of sheet-edge gripping chains, and a portion of one of the driving sprockets.

Fig. 6 is a transverse vertical section, 80 taken substantially on the line 6—6 of Fig. 5.

The glass sheet 1 is first drawn upwardly from the pool of molten glass 2 in receptacle 3. It is to be understood that the form of receptacle 3 here shown is merely illustrative, and that any other approved configuration or proportions could be given to this receptacle, and that usually means for heating the same will be provided to maintain the molten 85 glass 2 at the proper working temperature. Also any approved means, either within the molten glass or above the same, may be used to maintain sheet 1 to a fixed width at its source.

95 After sheet 1 has been conveyed from the vertical to the horizontal plane, as herein-after described, the sheet is carried away through suitable drawing and flattening mechanism, indicated generally at 4, into 100 the annealing leer. All of this may be as shown in systems now in use and need not be further described here.

105 Adjacent each side of the machine is mounted a suitable drawing and supporting mechanism for gripping and carrying the

edge portion only of the sheet from the vertical into the horizontal plane. These mechanisms are substantially identical with one another, except that portions thereof are reversed to fit the right and left hand portions of the sheet, and a description of one set of mechanism will suffice for both. An endless gripping and supporting chain 5 is carried by a driving sprocket 6 within one end of the chain loop and an idler sprocket 7 within the opposite end of the loop. Chain 5 may be of the usual sprocket type having teeth 60 on its inner face for engaging the teeth of the sprocket wheels, and having a somewhat uneven upper face 61 for insuring a positive grip upon the plastic glass sheet 1. Driving sprocket 6 is so positioned that the forward upwardly moving arc of the chain loop will be tangent to the vertical run of glass sheet 1, while the upper horizontal run of the chain loop will lie substantially in the same horizontal plane as the sheet-carrying surface of drawing and flattening mechanism 4. A second similar endless chain 8 is carried on suitable sprockets 9 and 10, so positioned that the lower run of chain 8 will travel over and parallel with that portion of the sheet-carrying run of chain 5 extending from the point of contact of sheet 1 therewith at the top of its vertical run to a point midway along the horizontal travel of sheet 1. The four chain-carrying sprockets 6, 7, 9 and 10, all lie in substantially the same vertical plane and are carried by the same supporting frame member 11. The shaft 12 of sprocket 6 is mounted in a fixed bearing 13 in this frame. Shaft 14 of driving sprocket 9 for chain 8, is mounted in a movable bearing 15. This bearing may be adjusted in the frame 11 by means of set-screws 16 to insure the proper spacing between the sheet-engaging runs of chains 5 and 8. The idler sprocket 7 at the opposite end of chain loop 5 is carried by a shaft 17 in bearing 18, slidably adjustable in one end of frame 11, by means of set-screw 19. The chain loop is tightened by suitably adjusting the screw 19. In the same manner the upper chain loop 8 is kept tight by adjusting the bearing 20 by means of screw 21.

A horizontal drive shaft 22 is mounted in bearings 23 at the lower edge of frame 11, and shaft 22 is provided with worms 24 and 25 which drive worm wheels 26 and 27 keyed to the outer ends of shafts 12 and 14 respectively.

A worm 28 at one end of shaft 22 meshes with and is driven by a worm 29 on vertical shaft 30, which in turn is driven through suitable worm gearing 31 from a horizontal drive shaft 32 extending in through one side of the machine. The supporting frame 11 is mounted on pivot 33 of a fixed supporting bracket 34 at the side of the ma-

chine. It will be noted that pivot 33 is coaxial with vertical drive shaft 30 so that the driving mechanism, above described, for the two driving sprockets will not be affected by any adjustment of supporting frame 11 about its pivot 33.

The vertical supporting member 35, at the opposite end of frame 11, is mounted in the arcuate groove 36 in fixed supporting bracket 37. The arcuate slot or groove 36 is concentric with pivot member 33. An adjusting screw 38, extending in through the side of the machine, engages the supporting member 35, and by suitably manipulating this screw the support 35 may be moved along the arcuate slot 36, whereby the angle which the vertical plane of the frame 11 and the gripping chains 5 and 8 makes with the side of the machine or with the center line of glass sheet 1 may be varied as desired. The frames 11 will ordinarily be so adjusted that the two sets of edge-gripping chains diverge from one another as they move forward with the sheet in the direction of the arrow, Fig. 1. In this way a constant lateral stretching tension will be applied to the glass sheet during the entire bending operation and during the first part of its horizontal run. This tension will overcome the tendency for the unsupported central portion of the sheet to sag and will at the same time draw out wrinkles or other surface variations which may have existed in the vertical run of the sheet.

At 39 is shown means whereby a blast of cold air, or other cooling fluid, may be blown against the lower idle run of chain 5 to cool the same prior to its engagement with the glass sheet. It is to be understood that any other form of cooling means might be used with either or both chain loops to keep them at the proper temperature.

It will be noted that the upper sheet-edge carrying run of chain 5 is slidably supported upon a horizontal trackway 40, formed as an extension of the frame 11. This will prevent sagging of the upper run of this chain and insure a flat horizontal travel for the glass sheet. The upper chain loop 8 is supported in its lower sheet-engaging run by the edge portion of the glass sheet, and the sprockets 9 and 10 will be so adjusted that the two chain loops will engage the sheet edge between them with sufficient pressure to positively grip the plastic sheet as indicated in Figs. 5 and 6. This will insure an effective hold upon the sheet edges during the lateral stretching operation as above described.

It will be noted that with this apparatus the main central portion of the glass sheet remains entirely untouched throughout its vertical run and until after the bending operation has been completed. Before the sheet comes into contact with any solid sup-

porting members in the horizontal plane, it has become set so that it is less liable to injury on its lower fire-polished surface.

Claims:

5. 1. That improvement in the art of drawing sheet glass, which consists in bending the sheet from one plane to another while unsupported except at its edges, by gripping the edge-portions of the sheet between members which move with the sheet throughout the bending operation.
10. 2. That improvement in the art of drawing sheet glass, which consists in bending the sheet from one plane to another while unsupported except at its edges, by gripping the edge-portions of the sheet between members which move with the sheet throughout the bending operation, and simultaneously forcing these gripping members to move along diverging paths so that lateral tension is applied to the glass sheet.
15. 3. That improvement in the art of drawing a continuous sheet of glass from a molten source, consisting in first drawing the sheet upwardly, and then bending the sheet into a substantially horizontal plane, while unsupported except adjacent its edges, the edge portions of the sheet being gripped while in its vertical run between means which move with the sheet throughout the bending operation.
20. 4. That improvement in the art of drawing a continuous sheet of glass from a molten source, consisting in first drawing the sheet upwardly, and then bending the sheet into a substantially horizontal plane, while unsupported except adjacent its edges, the edge portions of the sheet being gripped while in its vertical run between means which move with the sheet throughout the bending operation, the gripping means at opposite edges of the sheet moving away from one another during the bending operation to apply lateral tension to the glass sheet.
25. 5. In a sheet glass drawing apparatus, means for bending the sheet from one plane to another, comprising a continuous series of gripping elements engaging and moving with the sheet edges and supporting the same throughout the bending operation.
30. 6. In a sheet glass drawing apparatus,
7. In a sheet glass drawing apparatus, means for bending the sheet from the vertical to the horizontal plane, comprising a pair of cooperating chain-loops at each edge of the sheet, the sheet edge being gripped and carried between adjacent runs of the loops.
12. 8. In a sheet glass drawing apparatus, means for bending the sheet from the vertical to the horizontal plane, comprising a pair of cooperating chain-loops at each edge of the sheet, the sheet edge being gripped and carried between adjacent runs of the loops, and guiding means for the chain-loops whereby their sheet-engaging runs are caused to diverge and stretch the sheet laterally while it is being bent.
17. 9. In a sheet glass drawing apparatus, means for bending the sheet from the vertical to the horizontal plane, comprising a pair of cooperating chain-loops at each edge of the sheet, the sheet edge being gripped and carried between adjacent runs of the loops, guiding means for the chain-loops whereby their sheet-engaging runs are caused to diverge and stretch the sheet laterally while it is being bent, and means for adjusting the angle of divergence of the guiding means.
22. 10. In a sheet glass drawing apparatus, means for bending the sheet from the vertical to the horizontal plane, comprising a pair of cooperating chain-loops at each edge of the sheet, the sheet edge being gripped and carried between adjacent runs of the loops, a driving sprocket carrying one end of each loop, and an idler sprocket carrying the other end, a supporting frame in which all of the sprockets are mounted, and means for varying the inclination of this frame with respect to the center-line of the glass sheet.

Signed at Harrison, in the county of Hudson, and State of New Jersey, this 5th day of November, 1923.

JOHN C. HENDERSON.